

## UNITED STATES PATENT OFFICE

2,534,911

PROCESS OF REMOVING HYDROGEN EM-  
BRITTLEMENT OF BRIGHT NICKEL ELEC-  
TRODEPOSITSArthur S. Kasper, Detroit, Mich., assignor to  
Houdaille-Hershey Corporation, Detroit, Mich.,  
a corporation of MichiganNo Drawing. Application April 3, 1948,  
Serial No. 18,853

5 Claims. (Cl. 204—37)

**1**  
The present invention relates to a process of removing hydrogen embrittlement of bright nickel electrodeposits and more particularly to a process for the removal of hydrogen embrittlement of ductile bright nickel deposits caused by the subsequent electrodeposition over the nickel of chromium.

In the decorative chromium plating of steel or similar base metals, it is conventional to apply the chromium over an intermediate coating, such as a deposit of nickel, previously formed on the base metal. It has long been known that a large amount of hydrogen is evolved during the electrodeposition of chromium from chromium plating baths. As much as 35,000 volumes of hydrogen may be liberated at the cathode, or work, for each volume of chromium deposited. A portion of the hydrogen thus produced in the chromium plating operation is absorbed by the underlying nickel deposit and also by the base metal. In some instances, as will be pointed out, the absorption of hydrogen by the nickel deposit deleteriously affects the physical properties of the deposit.

Gray nickel deposits obtained by the use of Watts baths are ductile but require considerable buffing to obtain a mirror-bright coating suitable for subsequent chromium plating. The ductility of such buffed nickel deposits is not adversely affected by the occlusion of hydrogen by the nickel deposit and by the base metal during chromium plating.

Bright nickel deposits obtained by the use of modified Watts baths containing organic sulfur compounds or similar organic additives are bright but non-ductile as initially deposited, so that any embrittlement which may occur due to the occlusion of hydrogen during chromium plating produces no material change in the properties of the deposits. Bright nickel deposits produced as an alloy of cobalt and nickel are not believed to be embrittled during chromium plating. A process, however, which avoids the use of high percentages of cobalt will be more economical.

For these reasons, the occurrence of hydrogen embrittlement and the provision of methods for alleviating the harmful effects of such embrittlement have not assumed any great importance in the chromium plating industry. It has, however, been proposed in the literature that hydro-

**2**  
gen embrittlement be removed by heating a chromium plated object to a temperature sufficiently high to drive the occluded or absorbed hydrogen from the nickel layer and the base metal. The temperatures suggested by the prior art for this purpose have ranged from approximately 400° F. upward.

The copending application of W. E. Jenks, F. J. Fitzsimmons and Frank Ammermann, entitled "Method of and Bath Composition for Bright Nickel Plating," United States Serial No. 775,748, filed September 23, 1947, and assigned to the assignee of the present invention, discloses a bright nickel plating bath comprising an aqueous acid solution of nickel salts containing a minor amount of saccharin and coumarin. The nickel deposits obtained by the practice of the Jenks et al. disclosure are ductile and mirror-bright, requiring little or no polishing. Panels coated with such ductile bright nickel deposits may be bent or otherwise deformed beyond the elastic limit of the base metal without cracking or otherwise damaging the deposit. Such a combination of brightness and ductility has not been attained by the practice of the nickel plating processes of the prior art.

The ductile, mirror-bright nickel deposits of Jenks et al. are very desirable for use as an intermediate coating in chromium plating operations. However, it has been found that the ductile, bright nickel deposits of Jenks et al. readily absorb hydrogen during the chromium plating operation and that the occlusion of the hydrogen by the nickel deposit results in hydrogen embrittlement of the nickel layer. I have found that the ductility of the nickel deposit cannot be restored by heating the deposit to the temperatures disclosed in the prior art. The chromium layer, even when deposited upon the nickel plated surface as a very thin decorative coating, acts as a barrier to prevent the escape of the occluded hydrogen from the base metal and the nickel deposit. In order to impart sufficient energy to the entrapped hydrogen so that it may escape through the chromium barrier, it is necessary to heat the chromium plated object to temperatures ranging from 350° F. upwards. I have found that such heating adversely affects the ductility of the nickel deposit of Jenks et al. even though the occluded hydrogen is driven off. Temperatures low enough to avoid the thermal embrit-

lement of the nickel deposit are not sufficient to drive the hydrogen through the chromium layer to effectively restore the ductility of the nickel deposit.

The present invention now provides a process for removing hydrogen embrittlement from nickel deposits without causing further embrittlement of the deposit by excessive heating. I have discovered that ductile nickel deposits, such as those deposited upon a base metal as taught by the copending Jenks et al. application, may be heated to temperatures of about 300°-324° F. for a short period of time, or at lower temperatures for relatively long periods of time, without materially impairing the ductility of the deposit. I have also found that such temperatures are effective to remove absorbed hydrogen from the nickel layer and from the base metal in the absence of an all-enveloping chromium layer. Hydrogen embrittlement may be removed from a chromium plated object at relatively low temperatures by providing a non-chromium plated surface area on the object through which the absorbed hydrogen may pass. The absorbed hydrogen is relatively free to travel within the nickel deposit and the base metal and may be completely eliminated through any non-chromium plated area.

The process of the present invention therefore contemplates removing the hydrogen embrittlement of nickel deposits by subjecting the base metal and the nickel layer containing absorbed hydrogen to a temperature less than that temperature at which the nickel deposit becomes brittle. In the application of the process of the present invention to the removal of hydrogen embrittlement from deposits of nickel having a superimposed layer of chromium applied thereto, it is preferred that at least a portion of one surface of the chromium plated object be free of chromium so that the absorbed hydrogen may be eliminated from the article through that surface. This chromium-free surface of the object may be provided by either preventing the deposition of chromium on that surface or by removing the chromium from the surface after the entire article has been chromium plated.

It is, therefore, an important object of the present invention to provide a process for the removal of hydrogen embrittlement from bright nickel electrodeposits by subjecting the nickel deposits to a temperature sufficiently high to relieve hydrogen embrittlement but less than that temperature at which the nickel deposit becomes thermally embrittled.

It is another important object of the present invention to provide a method for removing hydrogen embrittlement of bright nickel deposits having a subsequently applied electrodeposit of chromium formed upon the nickel surface by providing a chromium-free portion of the nickel deposit through which the hydrogen may escape at temperatures less than those temperatures at which thermal embrittlement of the nickel layer occurs.

It is a further important object of the present invention to provide a process for removing hydrogen embrittlement from nickel deposits having a deposit of chromium applied thereon which comprises providing a surface free of chromium and heating the deposit to a temperature of about 300° F. or less to drive absorbed hydrogen through the non-chromium plated surface.

It is a still further object of the present inven-

tion to provide a process for the production of chromium plated objects having an intermediate layer of nickel free of hydrogen embrittlement which comprises depositing chromium from an electroplating bath upon said objects, subsequently removing the chromium deposit from at least a portion of the surface area of the object, and heating the plated object to a temperature of about 300° F. or less to drive absorbed hydrogen from the plated object and the nickel deposit.

It is a yet further important object of the present invention to provide a process for the chromium plating of nickel plated objects and the removal of hydrogen embrittlement of the nickel deposit which comprises the electrodeposition of chromium from a chromium plating bath upon said object while leaving a portion of the surface area of said object free of chromium and subsequently heating the plated object to a temperature of about 300° F. or less to remove absorbed hydrogen from the plated area and from the nickel deposit through the non-chromium plated surface area.

Other and further important objects of the present invention will be apparent from the disclosure in the specification and the appended claims.

The method of the present invention is particularly applicable to the removal of hydrogen embrittlement from ductile nickel deposits prepared by the process as taught by the above identified Jenks et al. application Serial No. 775,748. The broader ranges of proportions and ingredients and conditions of operation of the bath and method of Jenks et al. may be briefly summarized as follows:

|                                                           |       |                                 |
|-----------------------------------------------------------|-------|---------------------------------|
| Total nickel content                                      | ..... | 0.5 N-saturation                |
| Nickel chloride<br>(NiCl <sub>2</sub> .6H <sub>2</sub> O) | ..... | 0.1-1.5 N                       |
| Nickel sulphate<br>(NiSO <sub>4</sub> .7H <sub>2</sub> O) | ..... | 0.4 N-saturation                |
| Boric acid (H <sub>3</sub> BO <sub>3</sub> )              | ..... | 0-saturation                    |
| Citric acid                                               | ..... | 0-saturation                    |
| Saccharin (water<br>soluble)                              | ..... | 0.05-4.3 grams/liter            |
| Coumarin (C <sub>9</sub> H <sub>6</sub> O <sub>2</sub> )  | ..... | 0.01-1.3 grams/liter            |
| Temperature                                               | ..... | 60° F.-boiling                  |
| pH                                                        | ..... | 1.8-5.75                        |
| Current density (at plating<br>surface)                   | ..... | 16-144 amperes/ft. <sup>2</sup> |

The nickel deposits obtained by the practice of the Jenks et al. disclosure are bright, ductile, relatively free from internal tensile stress and possess excellent scratch hiding properties. It has been found that a steel plate having nickel deposited thereon by the method of Jenks et al. may be bent through an angle of 90° without cracking or otherwise damaging the nickel deposits. The occlusion of hydrogen during the chromium plating process results in a substantial reduction in the ductility of the bright nickel deposit obtained by the use of the Jenks et al. or any equivalent plating method. For example, the originally ductile plate following chromium plating initially exhibits cracking in the form of minute cracks upon bending at an angle of approximately 8 to 10°, but these minute cracks do not open further even when bent as far as 180°. By the process herein described, it is possible to restore the ductility of the Jenks et al. plate and to obtain a ductile coating of nickel and chromium.

I have found that if the article is chromium

plated all over, it is necessary to employ temperatures in the range of from 350 to 600° F. for periods of at least 30 minutes to drive off the absorbed hydrogen through the layer of chromium. Under such conditions, the nickel layer becomes embrittled by the severe heating and even though the absorbed hydrogen is driven off, the nickel deposits are not suitable for use when placed under stress due to thermal embrittlement. By the method of the present invention it is possible to drive off the absorbed hydrogen at temperatures much less than those of the prior art and to avoid overheating the nickel deposit to cause thermal embrittlement.

In accordance with the preferred process of the present invention, one surface or at least a portion of one surface of the nickel plated object is made chromium-free, either by not coating that surface with chromium during the chromium plating operation or by stripping a portion of the chromium layer from the nickel deposit or base metal. The deposition of chromium upon a nickel plated surface may be prevented during the chromium plating operation by means of a tightly fitting mask of suitable insulating material. Alternatively, a conductor in the form of a secondary cathode or "rubber" may be employed to prevent deposition of chromium upon a portion of the nickel plated surface. Any other suitable method of preventing deposition of chromium may be employed. If desired, the nickel plated article may be completely plated with chromium and the chromium removed from a portion of the surface by stripping, i. e. by the use of hydrochloric acid or other stripping agent, or by abrasion. The non-chromium plated area in the finished article may be sprayed with aluminum or other corrosion resistant material so that the exposed non-chromium plated area may be protected from corrosion.

Following the preparation of the chromium plated object with one surface or a portion of a surface free of chromium, the occluded hydrogen present in the nickel layer and in the base material may escape from the non-chromium plated surface. I have found that, while hydrogen embrittlement may be relieved by aging the plated article at room temperatures, an aging period of from 4 to 10 days is necessary to restore sufficient ductility to the nickel deposit. If more rapid removal of occluded hydrogen is desired, the nickel deposit may be heated to temperatures of about 300° F. or less to restore ductility to the deposit without causing appreciable thermal embrittlement. The time necessary for the restoration of ductility is an inverse function of the temperature, and in order to restore ductility within a reasonable time, I prefer to heat the deposit at temperatures of from 150 to 300° F. for periods of time ranging from several hours to 15 minutes.

The following examples will serve to illustrate the method of the present invention and the conditions under which the ductility of the nickel deposit may be restored.

#### EXAMPLE 1

Steel test panels were cleaned by a suitable procedure for use as test panels in this and the other examples given herein. An aqueous solution containing both nickel chloride and nickel sulfate was prepared. The total concentration of nickel in a bath was 2.9% N, the bath containing 0.4 N nickel chloride and 2.5 N nickel sulfate. The bath was prepared as follows: the desired

amounts of  $\text{NiCl}_2 \cdot 6\text{H}_2\text{O}$  and  $\text{NiSO}_4 \cdot 7\text{H}_2\text{O}$  were dissolved in water to give a 2.9 N nickel solution. The solution was maintained at a temperature of 125° F. 0.4 gram of coumarin per liter of solution was added to the solution by suspending the coumarin in a small amount, approximately 250 ml., of the nickel solution at a temperature of about 150° F., or above, and pouring the suspension into the larger body of solution. 0.25 gram of soluble saccharin per liter of solution was added by dissolving the proper amount in a small amount of water and adding the resulting solution to the nickel solution. Sufficient boric acid to give a 0.6 N solution (about 37.5 grams per liter) and sufficient citric acid to give a concentration of 1.0 gram per liter was added to the plating solution. The pH of the plating solution was maintained at a value of 3.9. The plates were plated in a solution at a current density of 64 amperes per square foot at the face of the panel. Following the removal of the nickel plated steel plates from the bath, the plates were heated at the indicated temperature for the time listed in Table I. To determine the ductility of the nickel plated steel plates, a simple bend test was employed. This test involves clamping the plate in a vise and bending it by striking it with a hammer. The piece was bent until cracking was observed and the amount of bending was determined. The results listed in Table I were obtained:

Table I

| Treatment Temperature | Treatment Duration | Amount of Bend Before Cracking |         |
|-----------------------|--------------------|--------------------------------|---------|
|                       |                    | Minutes                        | Degrees |
| Room temp.            | none               |                                | 90      |
| 300° F.               | 30                 |                                | 65      |
| 400° F.               | 30                 |                                | 25      |
| 500° F.               | 30                 |                                | 15      |

#### EXAMPLE 2

To determine the effect of aging time at room temperatures, steel plates, nickel plated in accordance with the disclosure of Jenks et al., as described in Example 1, were chromium plated in a conventional chromic acid-sulfate bath. Following the chromium plating operation, the layer of chromium was stripped from one surface of the plates by the use of a hydrochloric acid solution. The amount of bending was determined by a bend test as described in Example 1. The following results were obtained:

Table II

| Aging Time at Room Temperature | Amount of Bend Before Cracking | Degrees |      |
|--------------------------------|--------------------------------|---------|------|
|                                |                                | 5-8     | 8-10 |
| No aging                       |                                |         |      |
| After one day                  |                                |         |      |
| After four days                |                                |         |      |
| After six days                 |                                |         |      |
| After ten days                 |                                |         |      |

#### EXAMPLE 3

To determine the effect of time upon the amount of restored ductility, steel test panels plated as described in Example 1 were chromium plated and subjected to the conditions indicated in Table III. The chromium layer was stripped from one side of certain of the panels while the chromium layer on both sides was retained on certain reference panels.

The following results were obtained:

Table III

| Treatment Temperature | Duration of Treatment | Amount of Bend Before Cracking |                          |
|-----------------------|-----------------------|--------------------------------|--------------------------|
|                       |                       | Chromium Plated Both Sides     | Chromium Plated One Side |
| Room Temp.            | none                  | Degrees                        | Degrees                  |
| 300° F.               | 45 min.               | 5-8                            | 5-8                      |
| 300° F.               | 3 hrs.                | 5-8                            | 30                       |
|                       |                       |                                | 60                       |

## EXAMPLE 4

In order to determine more definitely the relief of hydrogen embrittlement by the process of the present invention, the ductility of nickel and chromium plated plates were tested by means of the Orlickson cup test. This test involves pressing a steel ball against a specimen so that the amount of deformation of the specimen may be measured up to the point that cracking of the deposit occurs. This test provides a means for definitely measuring and describing the ductility of a metallic coating. The following results were obtained by subjecting four specimens to the Orlickson cup test:

Specimen No. 1 was nickel plated as described in Example 1.

Specimen No. 2 was nickel and chromium plated as described in Example 2.

Specimen No. 3 was nickel and chromium plated as described in Example 2, the chromium layer was stripped from one surface, and the specimen was tested immediately after stripping.

Specimen No. 4 was prepared as specimen No. 3 and tested after heat relief at 300° F. for 30 minutes.

Table IV

| Specimen No. | Deformation |
|--------------|-------------|
| 1            | Inches      |
| 2            | 0.058       |
| 3            | 0.002       |
| 4            | 0.002       |
|              | 0.012       |

To summarize the process of the present invention by means of which hydrogen embrittlement of ductile bright nickel deposits may be relieved, occluded hydrogen is driven from the nickel layer by heating the plated object to a temperature less than that temperature at which the nickel deposit becomes thermally embrittled. The present invention is particularly applicable to the relief of hydrogen embrittlement of articles which have been chromium plated by the electrodeposition of chromium over nickel. The hydrogen entrapped in the nickel layer and the base material is expelled through a chromium-free surface of the plated object so that hydrogen embrittlement is greatly reduced. It is preferred that the plated object be heated to temperatures ranging from 150° F. to 300° F. in order to effect rapid removal of the hydrogen, although hydrogen embrittlement may be effectively removed by aging for relatively longer periods of time at room temperatures.

It will, of course, be understood that various details of the process may be varied through a wide range without departing from the prin-

ples of this invention and it is, therefore, not the purpose to limit the patent granted hereon otherwise than necessitated by the scope of the appended claims.

5 I claim as my invention:

1. A process for relieving hydrogen embrittlement of ductile bright nickel deposits formed as an intermediate layer on a metallic object and having a superimposed layer of chromium electrodeposited thereon, which comprises providing a chromium-free surface area on the plated object and subsequently heating the object to a temperature of from 150 to 300° F. for a period of time ranging from about 15 minutes to several hours, the specific period being correlated with the treating temperature with a shorter heating period being employed with higher temperatures.

2. The method of producing a ferrous foundation metal article having a relatively ductile nickel plate and a chromium plate thereover, which comprises electrodepositing a ductile, bright nickel plate on a ferrous foundation metal, electrodepositing chromium over a portion of said nickel electrodeposit and leaving another portion of said nickel surface exposed, and heating said article at a temperature of about 300° F. to expel hydrogen through said exposed nickel surface to relieve hydrogen embrittlement arising from said chromium electrodepositing step without thermally embrittling said nickel electrodeposit for a period of time ranging from about 15 minutes to several hours.

3. The method of producing a ferrous foundation metal article having a relatively ductile nickel plate and a chromium plate thereon, which comprises electrodepositing a ductile, bright nickel on a ferrous foundation metal from a bath containing nickel salts, coumarin and saccharin, electrodepositing chromium over said nickel electrodeposit, removing a portion of the chromium deposit to expose a portion of said nickel deposit and heating said article at a temperature of about 300° F. to expel hydrogen through said exposed portion of the nickel deposit to relieve hydrogen embrittlement arising from said chromium electrodepositing step without thermally embrittling said nickel electrodeposit for a period of time ranging from about 15 minutes to several hours.

50 4. In the method of producing a ferrous foundation metal article having a ductile nickel plate and a chromium plate thereon by the electrodeposition of a ductile, bright nickel deposit from a bath containing nickel salts, coumarin and saccharin and the electrodeposition of chromium on said nickel deposit, the steps which comprise stripping a portion of the chromium deposit from the plated article to expose a portion of said nickel surface and heating said article at a temperature of about 300° F. to expel hydrogen through said exposed nickel surface whereby hydrogen embrittlement arising from said chromium electrodepositing step is relieved without thermally embrittling said nickel electrodeposit for a period of time ranging from about 15 minutes to several hours.

5. In a method of producing a ferrous foundation metal article having a relatively ductile nickel plate and a chromium plate thereover by the electrodeposition of a ductile, bright nickel coating on a ferrous foundation metal and electrodepositing chromium over a portion of said nickel electrodeposit, the improvement which comprises preventing the electrodeposition of

chromium on a portion of said nickel surface to expose a portion of the nickel deposit and heating said plated article at a temperature of about 300° F. to expel hydrogen through the exposed portion of the nickel deposit whereby hydrogen embrittlement of the nickel deposit arising from said chromium electrodepositing step is relieved without thermally embrittling said nickel electrodeposit for a period of time ranging from about 15 minutes to several hours.

ARTHUR S. KASPER.

REFERENCES CITED

The following references are of record in the file of this patent:

UNITED STATES PATENTS

| Number    | Name            | Date          |
|-----------|-----------------|---------------|
| 154,435   | Adams           | Aug. 25, 1874 |
| 1,256,954 | Travers         | Feb. 10, 1931 |
| 1,792,082 | Fink et al.     | Feb. 10, 1931 |
| 1,795,384 | Von Busse       | Mar. 10, 1931 |
| 1,838,273 | McBride         | Dec. 29, 1931 |
| 1,857,929 | McFarland       | May 10, 1932  |
| 1,863,868 | McCullough      | June 21, 1932 |
| 1,963,391 | Wirshing et al. | June 19, 1934 |
| 2,270,316 | Kuhn et al.     | Jan. 20, 1942 |
| 2,291,590 | Lind et al.     | July 28, 1942 |
| 2,321,182 | Brown           | June 8, 1943  |

OTHER REFERENCES

Ser. No. 351,241, Weiner (A. P. C.), published May 18, 1943.